

July 25, 1961

J. E. CASCONE

2,993,802

FIBROUS ACOUSTICAL MEMBERS AND METHOD FOR PRODUCING THE SAME

Filed Sept. 23, 1957

5 Sheets-Sheet 1



FIG. 1.



FIG. 2.

FIG. 3.



FIG. 3.



FIG. 4.



FIG. 5.

INVENTOR.

John E. Cascone

BY

*Stalvin & Patterson*

ATTORNEYS

July 25, 1961

J. E. CASCONE

2,993,802

FIBROUS ACOUSTICAL MEMBERS AND METHOD FOR PRODUCING THE SAME

Filed Sept. 23, 1957

5 Sheets-Sheet 2



FIG. 6.

INVENTOR.

John E. Cascone

BY

*Staelin & Durman*

ATTORNEYS

July 25, 1961

J. E. CASCONE

2,993,802

FIBROUS ACOUSTICAL MEMBERS AND METHOD FOR PRODUCING THE SAME

Filed Sept. 23, 1957

5 Sheets-Sheet 3



FIG. 7

INVENTOR.  
John E. Cascone

BY  
*Stahl & Bernick*

ATTORNEYS

July 25, 1961

J. E. CASCONE

2,993,802

FIBROUS ACOUSTICAL MEMBERS AND METHOD FOR PRODUCING THE SAME

Filed Sept. 23, 1957

5 Sheets-Sheet 4



FIG. 8.

INVENTOR.

John E. Cascone

BY

*Stetson & Palmer*

ATTORNEYS

July 25, 1961

J. E. CASCONE

2,993,802

FIBROUS ACOUSTICAL MEMBERS AND METHOD FOR PRODUCING THE SAME

Filed Sept. 23, 1957

5 Sheets-Sheet 5



INVENTOR.

John E. Cascone

BY

*Stahl & Durman*

ATTORNEYS

1

2,993,802

## FIBROUS ACOUSTICAL MEMBERS AND METHOD FOR PRODUCING THE SAME

John E. Cascone, Granville, Ohio, assignor to Owens-Corning Fiberglas Corporation, a corporation of Delaware

Filed Sept. 23, 1957, Ser. No. 685,671  
8 Claims. (Cl. 117—26)

This invention relates to acoustical members of the type manufactured from compressed masses of fibrous glass and more particularly to such acoustical members having a coating which improves the soil resistance and appearance of such members as well as increasing their acoustical qualities.

Glass fiber acoustical board from which acoustical members are made is produced by densifying a blanket of heterogeneously arranged fibers. The fibers are formed by feeding a stream of molten glass to a high pressure steam or gas jet which shreds and attenuates the stream into fibers. The fibers are blown into a forming hood and collected on a conveyor below the hood as a blanket, say four to eight inches thick. Bonding resin is sprayed into the hood so that the fibers, or at least most of them, receive a coating of bonding resin, with the rate of feeding of the resin being so proportioned to the rate of fiber formation that only enough resin will be present on the average to bond the fibers together after densification.

While the majority of fibers formed in the process are deposited snugly in the accumulating mass, the currents of gas in the forming hood cause many of the fibers to be whirled and entangled into balls of fiber, called "snowballs" or "swirls." All such conglomerates fall onto and into the accumulating mass of fibers where their configuration causes a greater volume of space to be occupied by a given mass of fibers than when the fibers fall heterogeneously.

The blanket of fibers, with its uncured resin has an average apparent density of approximately 1½ to 2 pounds per cubic foot. The blanket is densified by being squeezed between the flights of the accumulating conveyor and an upper pressure conveyor which compact the mass to say ½ inch to 1 inch thickness, thus increasing its average apparent density to approximately 9 to 12 pounds per cubic foot. The densified mass is carried between the conveyors through a furnace to cure the bonding resin so that the fibers will be retained in the densified form as a board-like sheet when released from the conveyors.

Because of the resiliency of the fibers, they bulge into surface indentations in the conveyor flights during compaction and are cured in this shape so that the surfaces of the finished board are uneven, bearing an over-all pattern matching the conveyor surface configuration. Because sheets of this type are cut into boards, say 2 feet by 4 feet or into tiles, say 12 inches square, which are used as exposed wall and ceiling surfaces, this uneven pattern is not desirable. It is customary, therefore, to grind or sand one surface of the board until it is apparently smooth before subsequent treating steps.

This grinding or sanding step removes parts of the "snowballs" or "swirls" which have been flattened and exposes the ends of many fibers oriented in circular groups and extending at angles to the board surface. Because of the "snowball" configuration, the apparent density of the board at such areas is substantially less than the average apparent density of the board as a whole. These areas of low density cause many difficulties and are undesirable from all standpoints.

The larger interstices between fibers in such areas increase the air flow into and through the board which

2

greatly increases the air-borne dirt deposition at such areas and makes the board soiled unevenly. Further, these upstanding fibers cause the surface of the board to be rough and soil quickly when dirt laden air impinges thereon. If the board is painted or otherwise decorated for appearance sake, the larger interstices cause the board to soak up more paint at such areas. Since sound absorption of such boards is caused by the sound energy striking the resilient fibers, vibrating them and being converted to heat energy, the lower number of fibers in such areas results in a lowered acoustical efficiency.

Attempts have been made to overcome these deficiencies in several ways. Glass fiber acoustical boards and tiles have been covered by thin plastic films, fastened only at the edges, which provide an attractive surface appearance, prevent uneven soiling and yet transmit the sound energy into the interstices between the fibers and to the fibers themselves. Of course, the cost of the plastic film and the skilled labor necessary to adhere the film without wrinkles makes this type of acoustical member more costly.

Attempts have been made to coat the surface with paint selected to improve its appearance without interfering too greatly with the acoustical properties. The oriented low density areas, however, absorb the paint too readily, with the paint penetrating deeply into the interior of the mass. This considerably lessens the uniformity of soiling and acoustical properties and if the paint is in a heavy enough coating to make the soiling uniform, the acoustical properties are greatly lessened. It has been suggested that the surface characteristics may be improved from an appearance standpoint by first adhering a flat, swirl pattern, sheet of glass fibers to the surface of the board. This also spreads a net-work, as it were, over the lower density areas to level out the non-uniformities of soiling and acoustical properties. The cost of the sheets of fibers is high and they tend to delaminate, especially at the edges of the boards or tiles.

According to the invention, a densified glass fiber acoustical member is coated with a layer of a dispersion consisting of inexpensive, short particulate fibers in a liquid coating and film forming material. This coating is easily applied to the surface of the mass to form films which level out variations in soiling characteristics and improve acoustical properties while also providing a base for a second coating of paint designed to give the boards a pleasing appearance.

The principal object of the invention is to provide an improved glass fiber acoustical member having good resistance to soiling, good acoustical characteristics, and pleasing appearance.

It is a further object of the invention to provide a glass fiber acoustical member having a coating forming a multiplicity of minute sound transmitting films stretched between supporting fibers in the coating and in the board, the films acting to improve the acoustical properties of the coated member.

It is yet another object of the invention to improve the soiling characteristics of a glass fiber acoustical member by coating the exposed face with a coating which renders the air flow resistance of the board more nearly uniform over its entire surface and reduces the excessive deposition of air-borne dust and dirt which otherwise occurs in areas of low density.

Yet another object of the invention is the provision of a glass fiber acoustical member having a uniform, pleasing appearance.

Another object of the invention is to provide a method for fabricating improved glass fiber acoustical members having the properties outlined above and at low cost.

Other objects and advantages of the invention will be

apparent from the following detailed description of a preferred embodiment thereof, reference being made to the accompanying drawings, in which:

FIGURE 1 is a plan view of a portion of a densified glass fiber board showing a pattern on the surface of the board produced by the surface configurations of conveyors between which it is compressed.

FIG. 2 is an end view in elevation of the board shown in FIG. 1.

FIG. 3 is a fragmentary, enlarged, plan view of a portion of the board shown in FIG. 1, showing typical arrangements of the glass fibers of which the board is made.

FIG. 4 is a fragmentary, vertical sectional view on a further enlarged scale of a portion of the board shown in FIG. 3 and taken on the line 4—4,

FIG. 5 is a view similar to FIG. 4 but showing the board after a surface thereof has been ground or sanded smooth, the former surface being shown in broken lines,

FIG. 6 is a still further enlarged fragmentary plan view taken from the position indicated by the line 6—6 in FIG. 5 and showing some of the individual fibers both in the average heterogeneous arrangement and in the oriented arrangement of a "snowball" or "swirl,"

FIG. 7 is a fragmentary view in perspective on a still greater scale and showing a few of the fibers of the board with a first coating according to the invention freshly applied,

FIG. 8 is a view of the same area of a board as is illustrated in FIG. 7, after the first coating is dried,

FIG. 9 is a view similar to FIG. 8 but of another portion of the board shown in FIG. 6, with a first coating according to the invention,

FIG. 10 is a perspective view of a portion of a coated board showing the first coating after it is dried and including the area of FIG. 8, but on a much smaller scale,

FIG. 11 is a perspective view of the same portion of the board as in FIG. 10 and showing a second, decorative coating applied according to the invention to form a completed acoustical member,

FIG. 12 is a fragmentary vertical sectional view on an enlarged scale taken along the line 12—12 of FIG. 8 and showing a film formed by the first coating, and

FIG. 13 is a similar view of the film of FIG. 12, with a second coating applied according to the invention.

The figures of the drawing are intended to be approximate representations of a member and a coating therefor and the shapes, sizes, configurations, comparative scale, and arrangement of the fibers and coatings are only illustrative.

A portion of a densified glass fiber board suitable for fabrication into an acoustical member is generally indicated by the reference number 21 in FIGS. 1 and 2. The board 21 is made according to the process briefly described above and well known in the art.

As explained, when the soft mass of resin coated fibers, including "snowballs" and "swirls," is densified between converging conveyors and the resin is cured, the conveyor flights from irregularities on the surfaces 22 of the member 21, consisting of patterned protuberances 23 on the surfaces 22 between which a regular network of valleys 24 extends. Many of the fibers that would otherwise protrude from the surfaces 22 are squeezed into the surface during compaction and are held in that position when the binder is cured. As mentioned, the generally spherical "snowballs" are flattened into the board in the form of thin ellipsoids.

A smaller part of the portion 21 is shown in plan in FIG. 3 and in enlarged section in FIG. 4. The portion 21 is composed of a multiplicity of randomly disposed, individual glass fibers 25 which are accumulated in a plurality of generally defined planes approximately parallel to the main surface 22 of the portion 21. The part of the portion 21 shown in FIG. 3 comprises a group of swirled fibers 26 forming a "snowball," generally indicated at 27, which was compressed to a shallow ellipsoidal

shape (see also FIG. 5) when the glass fiber material was compacted.

After the densified board is cut into panels or tiles, the main surface 22 is ground or sanded down to remove the flight marks and assure that the upper and lower surfaces are parallel. The ground surface is indicated at 29 in FIG. 5. The grinding operation cuts across the "snowball" or "swirl" 27 and leaves many of the fibers 26 therein projecting at angles to the ground surface 29 of the board and forming an area of stubble, generally indicated at 28 in FIG. 5, in the ground surface 29 of the board 21. Some of the randomly disposed fibers are also cut off by the grinding although most of them lie in planes parallel to the surface and are either completely removed by the grinding or are not touched at all.

A greatly enlarged fragmentary view of a portion of the ground surface 29 of the board 21 as shown in FIG. 6. Most of the individual fibers, such as those designated 30, 31, 32, and 33, are randomly disposed, lying generally in planes parallel to the ground surface 29 on the board. Other fibers may form a "snowball" or "swirl" such as the "swirl" indicated at 34 comprising a multiplicity of conglomerated fibers 35 which extend at angles to the ground surface 29, the fibers 35 being ground off to leave ends 36 that form the stubble area. A few of the randomly disposed fibers may also extend at angles to the surface 29 with their ends 37 being cut off by grinding, but are insufficient in number to cause any difficulty.

Stubble areas are particularly deleterious for several reasons. The stubble produces a rough surface, even when coated with paint, that creates an unattractive appearance. The rough surface collects considerably more dirt or dust carried in moving air currents that impinge or contact the surface than do smoother surfaces and this further detracts from a pleasing appearance. The stubble areas also have a lower resistance to air flow with the result that more air tends to flow through these areas and further soil them. If these areas are heavily coated to provide a smoother surface and overcome these disadvantages, the sound absorption ability of the coated board will be seriously hampered.

Not only are these deleterious effects of the low density or stubble areas overcome by the coating of the invention but also the acoustical property of the board as a whole is better than that of a bare sanded board.

According to the invention, the coating on the ground surface 29 of the board consists of a first layer comprising a dispersion of minute, particulate fibers in a film-forming coating liquid and a second layer of a selected paint. A glass fiber board with such a coating on its surface constitutes the new acoustical member of the invention.

The liquid vehicle of the dispersion which forms the first layer has a film-forming constituent so that upon drying a plurality of small, permanent films are formed which stretch between and over the particulate fibers on the surface of the board and in some cases, between the main fibers of the fiber board. Vinyl compounds have been found suitable to be included to provide this result. A suspending agent or stabilizer may also be included to maintain the particulate fibers in suspension in the liquid vehicle to thereby minimize the necessity for stirring the dispersion. The dispersion may also include a pigment to impart color. It is preferred that the liquid vehicle of the first coating be immiscible with the resinous binder that is used to bond the glass fibers of the board in order to minimize penetration of the liquid into the interior of the board. Water has been found to be excellent as the liquid vehicle.

The particulate fibers employed in the dispersion are preferably of a natural mineral type. Organic fibers may promote the growth of fungi and glass fibers tend to settle and pack in the liquid vehicle and therefore do not spread well on the surface of the board. As-

bestos fibers are particularly useful because they maintain their fibrous qualities no matter how far they are broken down.

One dispersion that has been successfully applied to glass fiber acoustical boards contains asbestos fibers, the vast majority of which are less than  $\frac{1}{8}$  inch long and which constitute about 3½%, by weight, of the total dispersion. The dispersion also comprises, by weight, approximately 1 percent stabilizer, such as bentonite, about 3 to 4 percent film-former, such as polyvinyl acetate, about 5 percent light weight pigment, such as talc or the like; the remainder being water and an organic thickener, as Methocel or carboxy-methol-cellulose.

The dispersion may be sprayed onto the ground surface 29. Preferably, however, it is flooded on and its thickness controlled by a doctor blade. This procedure tends to spread a slightly heavier coat on those portions of the surface which have a lighter density or are rougher, such as the stubble area, generally indicated at 28 in FIG. 5.

A greatly enlarged view of the illustrated area of the board, and particularly of the fibers 30, 31, 32, and 33 is shown in FIG. 7 with a freshly applied first coating of the dispersion according to the invention. Asbestos fibers 38 to 44, inclusive, are randomly disposed over the glass fibers 30 to 33. In actual practice, however, the asbestos fibers may have diameters less than half the diameters of the glass fibers. The coating liquid forms films 45 to 50, inclusive, stretching between and over the asbestos fibers 38 to 44 and, in some instances, the glass fibers 30 to 33. These and similar films are formed over the entire surface of a board coated according to the invention. The films are formed by the film-forming constituent of the coating liquid, the stabilizer, and the pigment which constitute the layer covering the board surface. Although most films will be formed between asbestos fibers, for example, the films 47, 48, 49 and 50, some will be formed between glass fibers at the surface of the board, such as the films 45 and 46. In some instances no film will be formed, leaving openings in the coating, for example, the opening 51 delineated by asbestos fibers 40, 41, 43, and 42.

The freshly applied, first layer is then dried, in the particular instance by a convection furnace maintained at 400° F. in which the coated board or tile is placed for 1½ minutes. The heat causes the water in the coating liquid to evaporate and at the same time, causes the combination of the film-forming constituent, the stabilizer, and the pigment to shrink which may create pores in the layer thus formed. The films of FIG. 7 are shown after being dried in FIG. 8, where pores, such as a pore 52 in the film 45 and a pore 53 in the film 50 are shown. Other films may be more or less destroyed during drying to form openings where films formerly were, for example, such an opening being indicated by the reference number 46a, in FIG. 8. This is particularly true where the coating liquid is initially spread relatively thin between the fibers so that, after evaporation of the water and shrinkage of the other constituents, very little material remains. The surface tension of the liquid material tends to shrink the films toward the fibers.

All of the pores or openings through the first coating, whether originally existing, as the opening 51, formed by rupture of a film, as the pores 52 and 53, or resulting from destruction of a film as the opening 46a, function to pass sound energy into the interior of the board and through the intercommunicating interstices between the fibers to enable those fibers to vibrate and absorb the sound energy. The films are believed to intercept sound, vibrate by its energy, and re-transmit sound waves to fibers in the interior of the board. In addition, the vibration of the films causes fibers to which they are connected to be vibrated. However, the films may actually contain minute pores through which the sound is transmitted.

FIG. 9 is a view similar to FIG. 8 but showing films formed over a portion of the low density "swirl" 34 (see FIG. 6). Asbestos fibers 54 to 57 inclusive are supported principally on the ends 36 of the glass fibers 35 forming the "swirl" 34 and films 58 and 59 are shown as formed between the asbestos fibers 55, 56 and 57, and 54 and 55, respectively. These films are formed by the coating liquid and the film-forming constituent therein.

After the first dispersion coating is dried and the various films formed, a decorative paint is applied over the first coating. The paint may be of any conventional type but preferably is a type which is immiscible with and will not wet the binder used to bond the glass fibers together. The paint should also be immiscible with the first dispersion coating. A water-base, latex paint has been successfully used with the above-described dispersion. In practice, two coats of paint are separately applied and dried to give better control of the thickness of the paint coating than could be achieved with a single, heavier coating.

The paint layer is generally heavier than the fiber-containing first layer and flows relatively smoothly over the surfaces of the films, although the paint may form pores over some of the films. While the paint will close many of the pores in the first layer, control is exercised over the viscosity and quantity of the paint so that some of the pores are left at least partially open.

FIG. 10 shows a larger area of the board after the first layer has been dried, the area including the films 45 to 50 of FIG. 8 and the openings and pores 51, 52 and 53 as well as adjacent films and pores. In FIG. 11, the same area is shown after the second layer of two coats of paint is applied and dried. The board, the first layer of the dispersion of particulate fibers and coating liquid, and the second layer of paint, combined as shown here, constitute an acoustical member according to the invention. A surface 60 of the now finished acoustical member has a textured appearance containing a multiplicity of pores such as the pores 61, 62, and 63. The three finished pores 61, 62, and 63 are formed by the paint coatings in the original pores or openings 51, 52, and 53 respectively. As can be seen by comparing FIGS. 12 and 13, the pore 53 as originally formed in the film 50 is larger than the final pore 63 remaining after the coatings of paint, indicated at 64, are applied.

It has been found that approximately half as much paint is required for the new coating as for a coating utilizing a bonded sheet of glass fibers as previously described. Excellent sound absorption, soiling characteristics, and appearance are thus obtained with the new member using a lesser amount of paint.

Sound absorption, a primary consideration in acoustical members, is commonly measured in a room of known volume whose walls are of a smooth, dense substance having sound absorbing characteristics of a known, minute value. A sheet of the material to be tested, having a standard area of either 48 or 72 square feet, is placed in the room and sound is emitted thereto at a constant volume and at different, known frequencies. The time is measured for the sound to decay to a point where it is no longer audible, and theoretically to one millionth of its original intensity. A coefficient of sound absorption for the material being tested can then be obtained from known equations. Sound absorption coefficients are determined at frequencies of 125, 250, 500, 1000, 2000, and 4000 cycles per second. A numerical average of the four intermediate frequencies, 250, 500, 1000, and 2000, gives a value, known in the art as Noise Reduction Coefficient, or N.R.C.

It would ordinarily be expected that putting a coating on an acoustical board would reduce its N.R.C. value. However, with the new member, the films formed by the dispersion on the surface, which vary in area so that there is no chance of resonance occurring, are believed to intercept and absorb sound energy by vibrating and

may also pass sound through minute pores in the films. The films are also believed to transmit sound energy to the glass fibers and the minute fibers to which the films are attached, causing these fibers to vibrate more than would bare fibers, since without these films there would be considerably less area presented by these fibers for interception of the sound waves. Apparently for these reasons, the coating of the invention actually increases the N.R.C. value of a member an appreciable amount over that of a bare board of the same thickness.

The soiling characteristics of acoustical members is a second important consideration. There are two factors that cause non-uniformity of soiling: degree of surface roughness, which varies soiling by impingement of dirt laden air on the surface, and air flow resistance, which controls the amount and uniformity of air flow through the member. Soiling by impingement is particularly important around heating duct outlets in a ceiling. Heated air from the outlets partially impinges on adjacent portions of the ceiling, leaving dark areas of dirt around the edges of the outlets which create an unsightly appearance. The smoother the surface of the member, the less it will catch dust or dirt impinged thereon. The films formed by the new coating bridge rough portions, especially stubble, on the surface of the member and thus provide a smooth surface.

The second factor influencing the uniformity of soiling is air flow resistance. Air flow resistance of acoustical members is particularly important when the members are suspended in a room at a distance below a permanent ceiling to provide a false ceiling which creates a modern and attractive appearance in the room. In this position the acoustical members form two plenum chambers, one being a dead space between the permanent and false ceilings and one being the room below the false ceiling. The air pressure in the dead space between the permanent and the false ceilings is substantially constant while the air pressure in the room constantly varies due to such factors as the opening and closing of doors, wind blowing through open windows, and even the pumping action caused by the movement of elevators in their shafts. This varying pressure causes air to flow through the members, commonly known as "breathing," from the room to the dead space when the pressure in the room is higher than that in the dead space, and from the dead space to the room when pressure in the room is lower than that in the dead space. The acoustical members act as air filters during this movement of air and remove impurities from it, particularly at the surfaces of the members through which the air initially enters. Air flow from the room to the dead space causes the lower surfaces of the members to be covered with dust or dirt particles filtered from the air. A similar action takes place on the upper surfaces of the members as air flows from the dead space to the room, but this, of course, is unimportant from the standpoint of visible soiling.

When soiling occurs uniformly over the surfaces, the dirt is not apparent since it is present over the entire area and gradually darkens the members at a uniform rate. However, if there is greater air flow through some portions of the members than others, the dirt will accumulate faster at those portions because the greater volume of air carries a proportionately larger amount of dirt. The increased amount of dirt at those portions makes soiling considerably more noticeable since it will be in contrast to adjacent relatively clean areas having a higher resistance to air flow. Varying resistance to air flow in the members is caused by variations in apparent density at the "snow-balls" or "swirls." As explained, these variations are inherent in the production of glass fiber acoustical boards by the method outlined above.

The new acoustical member of the invention provides films formed by the dispersion which are impervious to air flow and also pores which, being randomly disposed, are generally constant in area and number for any given

surface area of a member which is reasonably large. The films and pores thus create a constant average resistance to air flow and tend to maintain uniform resistance and, hence, uniform soiling over the entire member.

Another phase of air flow resistance, in addition to uniformity, which influences soiling characteristics of an acoustical member, is the total resistance to air flow per unit of area. A greater over-all air flow resistance decreases the amount of air flowing through the member and, hence, the amount of dirt accumulated thereon.

Air flow resistance, besides affecting soiling due to breathing, as influenced by uniform and total air flow resistance, is usually related to soiling due to impingement. When the amount of coating on a board is increased, the surface usually tends to be smoother. Also, when the amount of coating is increased, the air flow resistance also increases. Thus, for a given acoustical member, air flow resistance, as influenced by the amount of coating, affects soiling from the standpoint of both impingement and breathing and as air flow resistance increases, soiling decreases.

The coating of the new acoustical member consisting of a glass fiber board and the dispersion and paint layers, may be applied more densely to create a smoother surface and a higher total air flow resistance of the acoustical member but without decreasing the acoustical absorption properties as will occur with other members when coatings are more densely applied to increase the air flow resistance. This has been proven by tests conducted to determine the N.R.C. of the new members having varying air flow resistances. Air flow resistance is measured by placing a 12 by 12 inch tile of the member transversely in a duct and passing air therethrough at a rate of 20 cubic feet per minute. The pressure differential upstream and downstream of the tile, in inches of water, is measured and constitutes the air flow resistance of the member. To illustrate, if a 12" x 12" tile of a member is placed in a 12 x 12 inch duct through which 20 c.f.m. of air is passed, and the pressure differential across the tile is 1.2 inches of water, the air flow resistance of the member is 1.2.

The results of a portion of these tests are as follows:

|                         | Air flow resistance | Frequency in cycles per second |     |     |       |       |       |        |
|-------------------------|---------------------|--------------------------------|-----|-----|-------|-------|-------|--------|
|                         |                     | 125                            | 250 | 500 | 1,000 | 2,000 | 4,000 | N.R.C. |
| Absorption coefficients |                     |                                |     |     |       |       |       |        |
| 45                      | .72                 | .08                            | .26 | .70 | .95   | .87   | .73   | .69    |
|                         | 1.10                | .09                            | .33 | .76 | .92   | .82   | .63   | .71    |
| 50                      | 2.20                | .08                            | .41 | .77 | .89   | .77   | .58   | .71    |

These figures show that air flow resistance of the acoustical member of the invention can be greatly increased without affecting the N.R.C. In the results shown, the air flow resistance was more than tripled without having any appreciable effect on the N.R.C. Although the absorption coefficients at the higher frequencies did decrease as the air flow resistance was raised, they increased at the lower frequencies which include the majority of noises produced in offices and the like.

The fact that air flow resistance can be greatly increased without affecting acoustical properties is particularly advantageous in the production of members according to the invention. An excessively heavy coating applied to a glass fiber board, although affecting air flow resistance, will not affect the acoustical absorption properties. Precise control of coating during production is therefore not essential to produce good acoustical members. Should any of a variety of factors produce an excessively heavy coating on the boards, they are still effective sound absorbers and need not be discarded.

The fact that air flow resistance of a given acoustical member can be increased to decrease the amount of soiling has been shown by actual tests. The amount of soiling of a member, due to impingement and breathing, is

measured in the art in terms of the amount of light reflected from the surface of the member before and after it is subjected to soiling, using air flow resistance as a standard of comparison. Nine 12 by 12 inch tiles cut from the member are first tested in their new, unsoiled state to determine the percent of light reflected from their surfaces. The tiles are then arranged in a square, three tiles on a side, and placed across a 3 by 3 foot duct at one side of which is a slot directed toward the upstream surface of a row of three tiles closest to the slot and designated as the first row. A second row of tiles is contiguous to the first row and disposed further from the slot, and a third row is contiguous to the second and adjacent the side of the duct opposite the side having the slot. Air containing a constant amount of dust or dirt is emitted through this slot at a velocity of one thousand feet per minute and impinges at a fixed angle on the upstream surface of the first row of tiles closest to the slot. Air is also passed axially through the duct at a sufficient rate to establish a pressure differential across the tiles of .03 inch of water. A narrow baffle is placed between the second and third rows of tiles and extends above the upstream surfaces of the tiles to prevent the air emitted from the slot from impinging on the third row. However, the dust in the air emitted from the slot that does not catch on the upstream surfaces of the first or second rows, passes above the baffle and is carried down through the third row of tiles by the air passing axially through the duct. The tiles are subjected to this test for three hours and are then again tested for light reflection. The greater the amount of dirt collected, the less will be the percent of light reflected. The difference between the percent of light reflected from the clean tile and the percent reflected from the soiled tile is a measure of the amount of soiling. The difference between the percents of light reflected from the first row of tiles, in their clean and soiled conditions, is due to the dust collected thereon from impingement and is dependent on the roughness of the surface. This difference in light reflection is the reflection loss due to impingement. The difference in light reflection for the third row, in the clean and soiled state, is due to the dust collected thereon from the air passing through the duct containing dust carried over from the impingement slot and is dependent on the air flow resistance of the tile. This difference in light reflection is the reflection loss due to breathing. The light reflection loss for the second row of tiles is due to a combination of breathing and impingement which is dependent on both air flow resistance and roughness.

Many soiling tests have been conducted according to the above described procedure on acoustical members made according to the invention. The results of three groups of nine tiles used in the above described acoustical test are shown below:

| Group  | Air flow<br>Resistance, inches<br>of water | Initial<br>Reflection,<br>percent | First Row<br>Reflection<br>loss due to<br>impinge-<br>ment, per-<br>cent | Third Row<br>Reflection<br>loss due to<br>breath-<br>ing, per-<br>cent |
|--------|--------------------------------------------|-----------------------------------|--------------------------------------------------------------------------|------------------------------------------------------------------------|
| 1----- | .72                                        | 82                                | 41                                                                       | 14                                                                     |
| 2----- | 1.00                                       | 82                                | 37                                                                       | 12                                                                     |
| 3----- | 2.10                                       | 83                                | 32                                                                       | 8                                                                      |

The test results show that soiling can be considerably decreased by increasing the air flow resistance of a given member. Increasing the air flow resistance from 1.72 to only 1.00 decreased the impingement loss almost ten percent and decreased the breathing loss more than fourteen percent. Soiling can be further decreased by further increasing the air flow resistance. Thus, with air flow resistance increased from 1.00 to 2.10 percent, the impingement loss decreased approximately fourteen percent and the breathing loss decreased approximately thirty-three percent. Of particular importance is the fact that the soiling can be decreased by increasing the air flow resistance

without decreasing the sound absorption of the new member. For the new members used in the above test, for example, the N.R.C. actually increased from .69 to .71 when the air flow resistance was increased from .72 to 2.10.

In addition to acoustical properties and soiling characteristics, appearance is an important consideration in the production of acoustical members. A textured appearance seems to be more pleasing to the eye than a smooth, even surface. It has been found that when air flow resistance (as measured by the above described test) of the new acoustical member is above approximately 1.6, the heavy coating will form an undesirably smooth surface. Because of the extremely smooth surface, impurities in the paint which would otherwise be hidden on a textured surface will be noticeable. This is particularly true in modern architecture in which windows are frequently extended to a point just below the ceiling. Light entering the upper portion of these windows further emphasizes impurities that tend to stand out from the smooth surface by creating a cross-lighting effect. To create a smooth appearance under such conditions, the paint must be initially free from impurities and must be dried in a carefully controlled, dust-free atmosphere. In addition, it has been found that as air flow resistance increases above 1.6, soiling due to the amount of air passing through a member changes very little. Consequently, the degree of soiling due to breathing or air flow is only slightly changed when the air flow resistance increases above 1.6. For these reasons, the thickness of the coating is controlled so as to maintain air flow resistance of the new member below 1.6.

At the same time, however, if the coating is too thin, so that the air flow resistance is below approximately .6, the surface of the member will be relatively lightly coated and will therefore be excessively rough so that soiling due to impingement will be very high. Thus, a coating producing an air flow resistance of the new member between .6 and 1.6 is preferred. Above this range the surface is smooth enough to show impurities in the paint, and below this range the surface is sufficiently rough so that soiling due to impingement is too high.

The above discussion has shown that the new acoustical member has many advantages. It enables higher and more uniform air flow resistance and smoother surfaces to be obtained to thereby decrease the degree of soiling and achieves these effects while providing high sound absorption which is not appreciably changed if an excessive amount of paint should be applied to the first coating. The new member also enables a given air flow resistance to be obtained with less paint. Thus soiling, as influenced by resistance to air flow, can be maintained at a minimum with less paint. Further, the new member is also inexpensive, easily manufactured, and the new coating does not tend to become separated from the surface of the glass fiber board.

The above has been intended to serve in an illustrative and not a limiting sense, the scope of the invention being only determined by the claims appended hereto.

I claim:

1. An acoustical member comprising a board having a generally planar main surface and consisting of a densified mass of heterogeneously arranged and spaced glass fibers bonded to each other by a resinous binder on said fibers, the heterogeneous arrangement of said glass fibers including glass fibers arranged generally in planes generally parallel to said main surface and conglomerates of other glass fibers, at least some of which extend angularly to said main surface, said densified mass having corresponding areas of different densities; and a discontinuous coating comprising a multiplicity of randomly disposed, inorganic, particulate fibers deposited from a liquid dispersion including a film-forming liquid onto said main surface of said board, said coating partially extending across spaces between said glass fibers at said

main surface of said board and being heavier in those areas of said board of lighter density, said coating forming a discontinuous film over said glass fibers bridging at least some of such spaces, at least in part.

2. An acoustical member comprising a board having a generally planar main surface and consisting of a densified mass of heterogeneously arranged and spaced glass fibers bonded to each other by a resinous binder on said fibers, the heterogeneous arrangement of said glass fibers including glass fibers arranged generally in planes generally parallel to said main surface and conglomerates of other glass fibers, at least some of which extend angularly to said main surface, said densified mass having corresponding areas of different densities; a discontinuous coating comprising a multiplicity of randomly disposed, inorganic, particulate fibers deposited from a liquid dispersion including a film-forming liquid onto said main surface of said board, said coating partially extending across spaces between said glass fibers at said main surface of said board and being heavier in those areas of said board of lighter density, said coating forming a discontinuous film over said glass fibers bridging at least some of such spaces, at least in part; and a second coating of pigmentitious material lying on at least part of the continuous portions of and across some of the gaps, at least in part, in the surface of said first coating.

3. An acoustical member comprising a board having a main surface and consisting of a densified mass of heterogeneously arranged and spaced fibers bonded to each other by a binder on said fibers, the heterogeneous arrangement of said fibers including fibers arranged generally in planes generally parallel to the main surface and conglomerates of other fibers, at least some of which extend angularly to said main surface; a discontinuous coating comprising a multiplicity of randomly disposed, particulate, inorganic fibers deposited from a liquid dispersion including a film-forming liquid onto said main surface of said board, said coating partially extending across spaces between said heterogeneously arranged and spaced fibers at said main surface of said board, said coating forming a discontinuous film over said heterogeneously arranged fibers bridging at least some of such spaces, at least in part; and a second coating of pigmentitious material lying on at least part of the continuous portions of and across some of the gaps, at least in part, in the surface of said first coating.

4. An acoustical member comprising a board having a generally planar main surface and consisting of a densified mass of heterogeneously arranged and spaced glass fibers bonded to each other by a resinous binder on said glass fibers, the heterogeneous arrangement of said glass fibers including glass fibers arranged generally in planes generally parallel to said main surface; a discontinuous coating comprising a multiplicity of randomly disposed, inorganic, particulate fibers deposited from a liquid dispersion including a film-forming liquid onto said surface of said board, said coating forming a discontinuous film over said glass fibers bridging at least some of the spaces between said glass fibers at said main surface of said board, at least in part; and a second coating of pigmentitious material lying on at least part of the continuous portions of the surface of said first coating and across some of the gaps in the surface of said first coating, said acoustical member having randomly disposed pores through both of said coatings.

5. An acoustical member comprising a board having a main surface and consisting of a densified mass of heterogeneously arranged and spaced glass fibers bonded

to each other by a binder on said fibers; a discontinuous coating comprising a film-forming carrier and a multiplicity of randomly disposed, particulate, inorganic fibers lying on said surface of said board, said coating forming

5 a discontinuous film over said heterogeneously arranged and spaced fibers bridging at least some of the spaces between said heterogeneously arranged and spaced fibers at said main surface of said board, at least in part; and a second coating of pigmentitious material lying on at least part of the continuous portions of the surface of said first coating and across some of the gaps in the surface of said first coating, said acoustical member having randomly disposed pores through both of said coatings.

15 6. The method for producing a coating on a fibrous board, said board comprising interbonded fibers and having a plurality of intercommunicating interstices between said fibers throughout its mass and surface gaps between those of said fibers forming the surface, said method comprising mixing a dispersion of minute, inorganic fibers in a film-forming liquid coating material, spreading a coating of said dispersion over the surface of the board to bridge at least a portion of said surface gaps between the board-forming fibers with said dispersion and to produce a multiplicity of randomly disposed films of varying area extending between some of said minute fibers and over portions of the surface of said board, and drying and shrinking said dispersion to form a multiplicity of pores through said coating.

30 7. The method for producing a coating on a fibrous board, said board comprising interbonded fibers having a plurality of intercommunicating interstices between said fibers throughout its mass and surface gaps between those of said fibers forming the surface, said method comprising mixing a dispersion of minute, inorganic fibers in a film-forming liquid coating material, spreading a coating of said dispersion over the surface of the board to bridge at least a portion of said surface gaps between the board-forming fibers with said dispersion and to produce a multiplicity of randomly disposed films of varying area extending between some of said minute fibers and over portions of the surface of said board, drying and shrinking said dispersion to form a multiplicity of pores through said coating, spreading paint over at least part of said films and over only some of said pores, and drying said paint.

45 8. In a method of forming an acoustical member from a board, said board comprising interbonded fibers having a plurality of intercommunicating interstices between said fibers throughout its mass and surface gaps between those fibers forming the surface, the improvement which comprises forming a multiplicity of films over at least a portion of said surface gaps, at least in part, forming a multiplicity of pores among at least some of said films, and applying a coating of paint over at least some of said films and over only some of said pores.

#### References Cited in the file of this patent

#### UNITED STATES PATENTS

|    |           |           |                |
|----|-----------|-----------|----------------|
| 60 | 1,370,666 | Novotny   | Mar. 8, 1921   |
|    | 2,609,321 | Patterson | Sept. 2, 1952  |
|    | 2,653,985 | Phillips  | Sept. 29, 1953 |
|    | 2,725,309 | Rodman    | Nov. 29, 1955  |
|    | 2,844,491 | Hubbard   | July 22, 1958  |

#### OTHER REFERENCES

Fiberglas Standards GL 6 Cl, July 1951, "Many forms for many uses."